

[54] DRY COMPOSITE BLENDED MAGNETIC DEVELOPER OF RESIN ENCAPSULATED FINE MAGNETITE AND RESIN ENCAPSULATED COARSE MAGNETITE

[75] Inventors: Nobuhiro Miyakawa; Masanori Fujii, both of Suita; Kouzi Maekawa, Kyoto, all of Japan

[73] Assignee: Mita Industrial Co. Ltd., Osaka, Japan

[21] Appl. No.: 324,652

[22] Filed: Nov. 24, 1981

[30] Foreign Application Priority Data

Nov. 27, 1980 [JP] Japan ..... 55-165828  
Dec. 2, 1980 [JP] Japan ..... 55-169151

[51] Int. Cl.<sup>3</sup> ..... G03G 9/08

[52] U.S. Cl. ..... 430/106.6; 430/111

[58] Field of Search ..... 430/106.6, 108, 110, 430/111

[56] References Cited

U.S. PATENT DOCUMENTS

2,965,573 12/1960 Gundlach ..... 430/108  
3,234,017 2/1966 Heyl et al. ..... 430/110  
3,520,811 7/1970 Swoboda ..... 252/62.54  
4,031,021 6/1977 Deming ..... 252/62.1  
4,142,981 3/1979 Bean et al. ..... 252/62.1  
4,165,393 8/1979 Suzuki et al. ..... 427/18  
4,218,530 8/1980 Lu ..... 430/107  
4,239,845 12/1980 Tanaka et al. ..... 430/122

4,272,600 6/1981 Sypula et al. ..... 430/106.6  
4,277,552 7/1981 Asanae et al. ..... 430/122  
4,311,779 1/1982 Miyakawa et al. ..... 430/107  
4,315,064 2/1982 Miyakawa et al. ..... 430/122  
4,331,757 5/1982 Tanaka et al. ..... 430/122  
4,345,014 8/1982 Oka et al. ..... 430/122  
4,362,803 12/1982 Miyakawa ..... 430/122

FOREIGN PATENT DOCUMENTS

2847768 10/1979 Fed. Rep. of Germany .  
55-28020 2/1980 Japan .  
2074745 11/1981 United Kingdom .

Primary Examiner—John E. Kittle

Assistant Examiner—John L. Goodrow

Attorney, Agent, or Firm—Sherman & Shalloway

[57] ABSTRACT

Disclosed is a dry composite magnetic developer consisting essentially of a particulate shaped article of a composition comprising a binder resin medium and a powdery magnetic material dispersed in the binder resin medium, wherein said developer is formed by dry blending (A) a first particulate shaped article comprising a non-pulverizing agglomerate of cubic particles of magnetite having a number average particle size of 1 to 10  $\mu\text{m}$  as measured by an electron microscope with (B) a second particulate shaped article comprising magnetite particles having a particle size of 0.2 to 1  $\mu\text{m}$  at an (A)/(B) weight ratio of from 95/5 to 10/90, especially from 95/5 to 30/70.

14 Claims, 2 Drawing Figures

*Fig. 1*



Fig. 2



**DRY COMPOSITE BLENDED MAGNETIC DEVELOPER OF RESIN ENCAPSULATED FINE MAGNETITE AND RESIN ENCAPSULATED COARSE MAGNETITE**

**BACKGROUND OF THE INVENTION**

**(1) Field of the Invention**

The present invention relates to an improvement in magnetic developers. More particularly, the present invention relates to a composite magnetic developer for electrophotography, which is excellent in the image density, the color hue, the image sharpness, the resolving power and the half tone-reproducing property.

**(2) Description of the Prior Art**

As the developer capable of developing an electrostatic latent image without using a particular carrier, there is known a so-called magnetic developer comprising a powder of a magnetic material contained in developer particles.

As one type of this one-component magnetic developer, there is known a so-called conductive magnetic developer in which a fine powder of a magnetic material is incorporated in developer particles to impart a property of being magnetically attracted and a conducting agent such as carbon black is distributed on the surfaces of the particles to impart them electrically conductive (see, for example, the specifications of U.S. Pat. No. 3,639,245 and U.S. Pat. No. 3,965,022). When this conductive magnetic developer is brought in the form of a so-called magnetic brush into contact with an electrostatic latent image-carrying substrate to effect development of the latent image, there can be obtained an excellent visible image free of a so-called edge effect or fog. However, as is well known, when the developer image is transferred to an ordinary transfer sheet from the substrate, a serious problem arises. More specifically, as described in Japanese Patent Application Laid-Open Specification No. 117435/75, when the inherent electric resistance of a transfer sheet used is lower than  $3 \times 10^{13} \Delta\text{-cm}$  as in case of plain paper, broadening of contour or reduction of the transfer efficiency is caused by scattering of developer particles at the transfer step. This disadvantage is moderated to some extent by coating the toner-receiving surface of the transfer sheet with a resin, wax or oil having a high electric resistance. This improvement, however, is reduced under a high-humidity condition. Furthermore, the cost of the transfer sheet is increased by coating with a resin or the like and the feel of the transfer sheet is reduced.

As another type of the one-component magnetic developer, there is known a non-conductive magnetic developer comprising an intimate particulate mixture of a fine powder of a magnetic material and an electroscopic binder. For example, the specification of U.S. Pat. No. 3,645,770 discloses an electrostatic photographic reproduction process in which a magnetic brush (layer) of the above-mentioned non-conductive magnetic developer is charged with a polarity opposite to the polarity of the charge of an electrostatic latent image to be developed by means of corona discharge, the charged developer is brought into contact with a latent image-carrying substrate to develop the latent image and the developer image is transferred onto a transfer sheet. This electrostatic photographic reproduction process is advantageous in that a transfer image can be formed even on plain paper as the transfer sheet. However, this process is still disadvantageous in that it

is difficult to uniformly charge the magnetic brush of the non-conductive magnetic developer even to the base portion thereof, it is generally difficult to form an image having a sufficient density and the apparatus become complicated because a corona discharge mechanism should be disposed in the developing zone.

Recently, there have been proposed a process in which an electrostatic latent image is developed by frictional charging of a non-conductive magnetic developer by frictional contact of the developer with the surface of a latent image-carrying substrate (see Japanese Patent Application Laid-Open Specification No. 62638/75) and a process in which development is effected by utilizing dielectric polarization of a non-conductive magnetic developer (see Japanese Patent Application Laid-Open Specification No. 133026/76). In the former process, however, if development conditions are not strictly controlled, fogging is readily caused (especially when the degree of the contact of the tip of the spike of magnetic toner particles with the surface of the photosensitive material is high) or fixing or blocking of the magnetic toner particles onto the developing sleeve is caused, and this undesirable phenomenon is especially conspicuous when the copying operation is conducted continuously. In the latter process, there does not arise the problem of fogging, but since a visible image is formed by developing a latent image by utilizing the dielectric polarizing effect induced in the magnetic toner, the low-potential area of the latent image is not effectively developed. Accordingly, in the resulting print, a low-density portion of an original is hardly reproduced and reproduction of a half tone is difficult. Moreover, prints obtained according to these two processes are poor in the image sharpness, and when a p-type photosensitive material such as selenium is used as the photosensitive plate and a positively charged image is developed, it is very difficult to obtain an image having a sufficient density according to any of the foregoing two processes.

Furthermore, the specification of U.S. Pat. No. 4,102,305 discloses a process in which a one-component type magnetic developer, the electric resistance of which changes depending on the intensity of the electric field, namely a one-component type magnetic developer which becomes substantially conductive in a high electric field but has a high electric resistance in a low electric field, is used, a high voltage is applied between a magnetic brush-forming sleeve and a photosensitive plate to effect development under such conditions that the developer particles become conductive and transfer of the developer particles to a transfer sheet is carried out in a low electric field or in an electric field-free state to obtain an excellent transferred image. This specification teaches that the above-mentioned developer having a high electric field dependency of the electric resistance is prepared by spray-granulating 50% by weight of stearate-coated magnetite and 50% by weight of a styrene/n-butyl methacrylate copolymer. This process is excellent in the above idea of obtaining a good transferred image, but this process is disadvantageous in that a peculiar high voltage apparatus is necessary for the development and though the formed image has a high density, the image sharpness is still insufficient.

Moreover, the specification of U.S. Pat. No. 4,121,931 discloses a process in which an electrically insulating one-component type magnetic developer is

used, a magnetic brush-forming sleeve is used as an electrode and a voltage is applied between this electrode and a photosensitive plate to cause a turbulent agitation in the developer on the sleeve, whereby the developer particles are uniformly charged. This process, however, is disadvantageous in that a high voltage apparatus should be disposed in the developing zone and special means should be disposed to agitate the developer particles on the sleeve.

As will be apparent from the foregoing description, the conventional researches made on one-component type magnetic developers and developing processes using these developers are concentrated to the composition of the developer, the developer-preparing process and the process for charging developer particles, but properties of magnetite to be incorporated into the developer have hardly been studied.

Ordinarily, when a magnetic brush of a one-component type developer is brought into contact with the surface of an electrostatic latent image-carrying substrate, the individual developer particles receive an electrostatic attracting force (Coulomb force) acting between the developer particles and the electrostatic latent image and a magnetic attracting force acting between the developer particles and a magnetic brush-forming magnet. The developer particles on which the Coulomb force is larger are attracted to the electrostatic latent image, while the developer particles on which the magnetic attracting force is larger are attracted to the magnetic sleeve, with the result that development is effected according to the electrostatic latent image on the substrate. Therefore, it is required for the one-component type magnetic developer that a certain balance should be maintained between magnetic characteristics and charging characteristics at the development step. Accordingly, it will readily be understood that the characteristics of the magnetic material powder used for the one-component type magnetic developer have important influences on the characteristics of an image which will be formed.

#### SUMMARY OF THE INVENTION

In accordance with the present invention, there is provided a dry composite magnetic developer consisting essentially of a particulate shaped article of a composition comprising a binder resin medium and a powdery magnetic material dispersed in the binder resin medium, wherein said developer is formed by dry blending (A) a first particulate shaped article comprising a non-pulverizing agglomerate of cubic particles of magnetite having a number average particle size of 1 to 10  $\mu\text{m}$  as measured by an electron microscope with (B) a second particulate shaped article comprising magnetite particles having a particle size of 0.2 to 1  $\mu\text{m}$  at an (A)/(B) weight ratio of from 95/5 to 10/90, especially from 95/5 to 30/70.

#### BRIEF DESCRIPTION OF THE DRAWINGS

FIG. 1 is an electron microscope photograph of the powdery magnetic material consisting of a non-pulverizing agglomerate of cubic particles, which is used for the first developer component in the present invention.

FIG. 2 shows an X-ray diffraction pattern of the agglomerate shown in FIG. 1.

#### DETAILED DESCRIPTION OF THE PREFERRED EMBODIMENTS

The magnetic developer of the present invention is characterized in that the above-mentioned two kinds of particulate shaped articles (resin-magnetic material particulate shaped articles) comprising powdery magnetic materials different from each other are used in the dry-blended state. When the above-mentioned non-pulverizing agglomerate of magnetite particles is used as the magnetite of the first developer component, the image sharpness and resolving power can highly be improved over the conventional one-component type magnetic developers including magnetite of the needle or cubic crystal form or amorphous magnetite, and furthermore, the reproducibility of a half tone can also be improved. When the above-mentioned first developer component (first particulate shaped article) is dry-blended at a specific weight ratio with a second developer component (second particulate shaped article) comprising fine magnetite particles having a particle size of 0.2 to 1  $\mu\text{m}$ , the image density can be improved remarkably over the image density attained when either of the first and second developer components is singly used, and the color hue of the formed image can be made purely black or substantially purely black.

As is seen from the electron microscope photograph of FIG. 1 and the X-ray diffraction pattern of FIG. 2, the powdery magnetic material used for the first developer component in the present invention is magnetite consisting of a one-pulverizing agglomerate of cubic particles.

By the term "non-pulverizing agglomerate" used in the instant specification and appended claims is meant an agglomerate of fine particles which are densely aggregated with one another as shown in FIG. 1 and in which the particle size distribution is not substantially changed even by an ordinary pulverizing treatment, for example, 5 hours' ball-milling treatment.

This non-pulverizing agglomerate has a number average particle size of 1 to 10  $\mu\text{m}$ , especially 2 to 7  $\mu\text{m}$ , as measured by an electron microscope. Namely, it has a particle size larger than the particle size of ordinary magnetite particles.

Since the magnetic material used for the first developer component in the present invention has the above-mentioned dense aggregate structure and a relatively coarse particle size, the volume per unit weight, namely the bulk, is smaller than that of particles of magnetite of the cubic or needle crystal form or amorphous magnetite heretofore used for one-component magnetic developers. Accordingly, in the first magnetic developer component of the present invention, the resin/magnetite volume ratio can be made much higher than that in the conventional one-component type magnetic developers when the comparison is made based on the same weight ratio of magnetite. Accordingly, as will readily be understood, in the first magnetic developer component of the present invention, much higher inherent charging characteristics can be given to the resin.

It has been known that a polymeric material having a larger dielectric constant is more readily positively charged (see The Society of Photographic Scientists and Engineers, 2nd Int. Conf., 1974, pages 95 to 100). It has been found by us that in a magnetic developer comprising a powdery magnetic material dispersed in a binder medium, if the dielectric constant of the magnetic developer is small, it is likely to be negatively

charged by friction, and that if the dielectric constant is large, the magnetic material is likely to be positively charged by friction. More practically, developer particles comprising magnetite in an amount of 55% by weight based on the total developer have a dielectric constant of 3.85 to 4.05, whereas magnetic developer particles comprising 55% by weight of the above-mentioned non-pulverizing agglomerate of cubic particles have a dielectric constant of 3.79. Accordingly, it has been confirmed that the magnetic developer of the present invention is more readily negatively charged.

As pointed out hereinbefore, the powdery magnetic material used for the first developer component in the present invention has a smaller bulk, that is, a larger apparent density, than ordinary magnetite. More specifically, the powdery magnetic material has an apparent density of 0.5 to 1.5 g/ml, especially 0.7 to 1.3 g/ml, as determined according to the method of JIS K-5101.

The non-pulverizing agglomerate of cubic particles has magnetic characteristics of a saturation magnetization of 75 to 88 emu/g, a residual magnetization of 3 to 12 emu/g and a coercive force of 40 to 150 Oe.

The non-pulverizing agglomerate of cubic particles used in the present invention is prepared according to the following method, through an applicable method is not limited to this method.

A weakly alkaline aqueous solution, for example, aqueous ammonia, is added to an aqueous solution of iron (III) sulfate to form precipitates of iron (III) hydroxide. The precipitates are subjected to a hydrothermal treatment under pressure while maintaining the pH value of the mother liquor at 3 to 9, whereby gel-like precipitates of iron hydroxide are changed to cubic particles of alpha- $\text{Fe}_2\text{O}_3$  (Hematite). If the weakly alkaline aqueous solution is used to maintain the pH value of the mother liquor to a level close to the acidic side, fine cubic particles which tend to aggregate are formed, and the so-obtained particles are aged by carrying out the hydrothermal treatment at 150° to 230° C. for a long time, for example, more than 50 hours, whereby alpha-diiron trioxide having the configuration specified in the present invention can be obtained. If this alpha-diiron trioxide is reduced under known conditions, for example, by heating it at 400° C. with hydrogen in a reducing furnace, triiron tetroxide ( $\text{Fe}_3\text{O}_4$ ) having the configuration specified in the present invention can be obtained. The reducing treatment is ordinarily carried out so that the  $\text{Fe}^{2+}/\text{Fe}^{3+}$  atomic ratio is in the range of from 0.9/1.0 to 1.1/1.0. Thus, triiron tetroxide having the above-mentioned specific fine-structure can be obtained.

The X-ray diffraction pattern of the agglomerate type magnetite used in the present invention is the same as that of ordinary magnetite of the cubic crystal form and in view of the height of the diffraction peak, it has been confirmed that the magnetite used in the present invention is not substantially different from ordinary magnetite of the cubic crystal form in the degree of crystallization.

As the binder medium for dispersing this non-pulverizing agglomerate of cubic particles, there can be used resins, waxy materials or rubbers which show a fixing property under application of heat or pressure. These binder medium may be used singly or in the form of a mixture of two or more of them. It is preferred that the volume resistivity of the binder medium be at least  $1 \times 10^{15} \Omega\text{-cm}$  as measured in the state where magnetite is not incorporated.

As the binder medium, there are used homopolymers and copolymers of mono- and di-ethylenically unsaturated monomers, especially (a) vinyl aromatic monomers and (b) acrylic monomers.

As the vinyl aromatic monomer, there can be mentioned monomers represented by the following formula:



wherein  $\text{R}_1$  stands for a hydrogen atom, a lower alkyl group (having up to 4 carbon atoms) or a halogen atom,  $\text{R}_2$  stands for a substituent such as a lower alkyl group or a halogen atom, and  $n$  is an integer of up to 2 inclusive of zero, such as styrene, vinyl toluene, alpha-methylstyrene, alpha-chlorostyrene, vinyl xylene and vinyl naphthalene. Among these vinyl aromatic monomers, styrene and vinyl toluene are especially preferred.

As the acrylic monomer, there can be mentioned monomers represented by the following formula:



wherein  $\text{R}_3$  stands for a hydrogen atom or a lower alkyl group, and  $\text{R}_4$  stands for a hydroxyl group, an alkoxy group, a hydroxyalkoxy group, an amino group or an aminoalkoxy group, such as acrylic acid, methacrylic acid, ethyl acrylate, methyl methacrylate, butyl acrylate, butyl methacrylate, 2-ethylhexyl acrylate, 2-ethylhexyl methacrylate, 3-hydroxypropyl acrylate, 2-hydroxyethyl methacrylate, 3-aminopropyl acrylate, 3-N,N-diethylaminopropyl acrylate and acrylamide.

As another monomer to be used singly or in combination with the above-mentioned monomer (a) or (b), there can be mentioned, for example, conjugate diolefin monomers represented by the following formula:



wherein  $\text{R}_5$  stands for a hydrogen atom, a lower alkyl group or a chlorine atom, such as butadiene, isoprene and chloroprene.

As still another monomer, there can be mentioned ethylenically unsaturated carboxylic acids and esters thereof such as maleic anhydride, fumaric acid, crotonic acid and itaconic acid, vinyl esters such as vinyl acetate, and vinyl pyridine, vinyl pyrrolidone, vinyl ethers, acrylonitrile, vinyl chloride and vinylidene chloride.

It is preferred that the molecular weight of such vinyl type polymer be 3,000 to 300,000, especially 5,000 to 200,000.

In the present invention, it is preferred that the above-mentioned agglomerate be used in an amount of 35 to 75% by weight, especially 40 to 70% by weight, based on the sum of the amounts of the binder medium

and the magnetic material. Magnetite is uniformly and homogeneously kneaded with the binder medium and the kneaded composition is granulated, whereby the intended first magnetic developer component is obtained.

Known auxiliary components for developers may be added according to known recipes prior to the above-mentioned kneading and granulating steps. For example, pigments such as carbon black and dyes such as Acid Violet may be added singly or in combination in amounts of 0.5 to 5% by weight based on the total composition so as to improve the hue of the developer. Furthermore, a filler such as calcium carbonate or powdery silica may be added in an amount of up to 20% by weight based on the total composition to obtain a bulk-ing effect. In the case where fixing is effected by a heat roll, an offset-preventing agent such as a silicone oil, a low-molecular-weight olefin resin or a wax may be used in an amount of 2 to 15% by weight based on the total composition. In the case where fixing is effected by means of a pressure roll, a pressure fixability-improving agent such as paraffin wax, an animal or vegetable wax or a fatty acid amide may be used in an amount of 5 to 30% by weight based on the total composition. Furthermore, in order to prevent cohesion or agglomeration of developer particles and improve the flowability thereof, a flowability-improving agent such as a fine powder of polytetrafluoroethylene or finely divided silica may be added in an amount of 0.1 to 1.5% by weight based on the total composition.

Shaping of the developer can be accomplished by cooling the above-mentioned kneaded composition, pulverizing the composition and, if necessary, classifying the pulverization product. Mechanical high-speed stirring may be conducted so as to remove corners of indeterminate-shape particles.

It is ordinarily preferred that the number average particle size of the developer particles be in the range of 5 to 35 microns and be at least 2 times the number average particle size of the agglomerate particles, though the particle size of the developer particles is changed to some extent according to the intended resolving power. The first developer component comprising indeterminate-shape particles formed by kneading and pulverization according to the present invention exerts enhanced effects of increasing the transfer efficiency and elevating the image sharpness.

In the present invention, the first magnetic developer component (A) containing the above-mentioned agglomerate type magnetite is combined with the second magnetic developer component (B) comprising fine magnetite particles having a particle size of 0.2 to 1  $\mu\text{m}$  at an (A)/(B) weight ratio of from 95/5 to 10/90, preferably from 95/5 to 30/70, especially preferably from 90/10 to 40/60. When both the developer components are combined at the above-mentioned weight ratio and used, the image density is highly improved over the image density attainable by single use of either of the two components. Moreover, this increase of the image density can be attained without impairing the advantages of the non-pulverizing agglomerate of magnetite. The developer component comprising the non-pulverizing agglomerate of magnetite is especially suitable for attaining the objects of improving the image sharpness, resolving power and half tone-reproducing property. However, this developer component is still insufficient in that an image of a color hue deviating from pure black, that is, a slightly brownish black, is often given.

According to the present invention, by combining this developer component comprising the agglomerated magnetite with the second developer component comprising magnetite having a fine particle size, an image having a pure-black color or substantially pure-black color can be obtained.

Magnetite of the needle or cubic crystal form or amorphous magnetite can optionally be used as the magnetite of the second developer component if the particle size is in the range of from 0.2 to 1  $\mu\text{m}$ , preferably from 0.3 to 0.8  $\mu\text{m}$ . Such form of magnetite depends on the crystal form of starting  $\alpha$ -diiron trioxide (hematite).

Ordinary fine magnetite particles have a large bulk because the particle size is fine, and the apparent density is in the range of from 0.2 to 0.45 g/ml as determined according to the method of JIS K-5101.

In a preferred embodiment of the present invention, magnetite which has such a high apparent density as exceeding 0.45 g/ml though the number average particle size is not larger than 1 micron, especially in the range of from 0.1 to 0.7 micron, is used as the magnetite for the second developer component. In ordinary magnetite, the apparent density tends to decrease with reduction of the particle size. If magnetite particles having a fine particle size and a small apparent density are incorporated in the second developer component and this second developer component is used in combination with the first developer component containing the above-mentioned agglomerate of magnetite particles, the object of obtaining an image having a pure-black color or substantially pure-black color can be attained. However, in this case, the object of improving the image density at high-speed development is not satisfactorily attained. Namely, if development is carried out at a high speed by using the above composite developer, the image density is lower than the image density obtained when development is carried out at a low speed. In contrast, according to the above-mentioned preferred embodiment of the present invention, by selecting specific magnetite having a fine particle size and a relatively large apparent density and incorporating this magnetite into the second developer component and combining this second developer component with the first developer component comprising the above-mentioned agglomerate of magnetite particles, a magnetic developer which can be applied to high-speed development, that is, high-speed reproduction, can be provided and prominent increase of the image density at high-speed development can be attained without impairing the advantages attained by the non-pulverizing agglomerate of magnetite contained in the first developer component. Moreover, this composite developer is advantageous in that both the components are consumed at the same speed and the initial composition is not substantially changed while the composite developer is used.

The fine magnetite used in the above-mentioned preferred embodiment consists ordinarily of cubic particles and/or slightly rounded indeterminate-shape particles, and the shape anisotropy defined as the ratio of the maximum size to the minimum size is in the range of from 1.0 to 5.5, preferably from 1 to 3.

The fine magnetite particles used in the above-mentioned preferred embodiment are prepared according to the following method, though an applicable method is not limited to this method.

An alkaline aqueous solution of sodium hydroxide is added to an aqueous solution of iron (III) sulfate to form

precipitates of iron (III) hydroxide. The precipitates are subjected to a hydrothermal treatment under pressure while maintaining the pH value of the mother liquor at 4 to 11, whereby gel-like precipitates of iron hydroxide are changed to cubic particles of  $\alpha$ -Fe<sub>2</sub>O<sub>3</sub> (hematite). Conditions for the preparation of this cubic  $\alpha$ -diiron trioxide are described in detail, for example, in Nobuoka et al., Kogyo Kagaku Zasshi, 66, page 412 (1963). The hydrothermal treatment may be carried out at a temperature of 150° to 230° C. for 10 to 100 hours. Ordinarily, a higher pH value of the mother liquor results in a larger particle size. If not only the pH value of the mother liquor but also the treatment temperature and the treatment time are appropriately adjusted,  $\alpha$ -diiron trioxide having a predetermined particle size is obtained. If this  $\alpha$ -diiron trioxide is reduced under known conditions, for example, by heating it at 400° C. with hydrogen in a reducing furnace, triiron tetroxide (Fe<sub>3</sub>O<sub>4</sub>) having a cubic crystal form or a slightly rounded indeterminate-shape can be obtained. The reducing treatment is ordinarily carried out so that the Fe<sup>2+</sup>/Fe<sup>3+</sup> atomic ratio is in the range of from 0.9/1.0 to 1.1/1.0. Thus, triiron tetroxide having the above-mentioned characteristics can be obtained.

In preparation of the above-mentioned  $\alpha$ -diiron trioxide as the precursor, if the hydrothermal treatment is carried out at a relatively low pH value, magnetite having a slightly rounded amorphous shape where corners of cubes are removed is obtained. Such magnetite particles can be used in the present invention as well as magnetite particles of the cubic crystal form.

The preparation of the second developer component (B) comprising fine magnetite particles is carried out in the same manner as described hereinbefore with respect to the first developer component (A) comprising agglomerate type magnetite particles. More specifically, the above-mentioned binder media and additives are used in the above-mentioned proportions. Of course, in the preparation of the second developer component (B), the kind or mixing ratio of the resin may be changed from that adopted in the preparation of the first developer component. Moreover, omission of an additive used for the first developer component (A) or addition of an additive not used for the first developer component (A) may optionally be made in preparing the second developer component (B).

It is preferred that the particle size of the second developer component (B) be smaller than that of the first developer component (A) and be in the range of from 5 to 30 microns.

The product of the present invention can be obtained by dry-blending the first developer component (A) with the second developer component (B) according to known dry-blending procedures.

In the electrostatic photographic reproduction process using the developer according to the present invention, formation of an electrostatic latent image can be performed according to any of the known methods. For example, an electrostatic latent image can be formed by uniformly charging a photoconductive layer formed on a conductive substrate and subjecting the photoconductive layer to imagewise exposure.

A visible image of the developer is formed by bringing a magnetic brush of the above-mentioned composite magnetic developer into contact with the electrostatic latent image-carrying surface of the substrate.

Development of the electrostatic latent image with the developer of the present invention can be accom-

plished, for example, according to the following procedures. The above-mentioned one-component type magnetic developer is charged in a developer hopper. A non-magnetic sleeve is rotatably mounted on a lower end opening of the hopper, and a magnet is disposed in the interior of the sleeve so that the magnet turns in a direction opposite to the rotation direction of the sleeve. When the sleeve and magnet are rotated, a brush layer of the magnetic developer is formed on the sleeve, and this brush layer is cut into an appropriate length by a spike-cutting plate. Then, the brush layer of the developer is lightly contacted with a selenium drum which is rotated in the same direction as the rotation direction of the sleeve to develop an electrostatic latent image on the selenium drum with the magnetic developer.

Then, the developer image on the substrate is brought into contact with a transfer sheet, and corona charging is effected from the back surface of the transfer sheet with the same polarity as that of the electrostatic latent image, whereby the developer image is transferred onto the transfer sheet.

In the present invention, fixation of the transferred image may be carried out according to any of a heat roller fixation method, a flash lamp fixation method and a pressure roller fixation method, and an appropriate fixation method is selected according to the kind of the developer.

The developer of the present invention is especially effective for a p-type photosensitive plate on which a positively charged latent image is formed, for example, a selenium photosensitive plate or a photosensitive plate comprising an organic photoconductive material layer. The conventional one-component magnetic developer of the frictional charging type can be applied to a photosensitive plate having a negatively charged latent image, but if this developer is used for developing a positively charged latent image formed on the above-mentioned p-type photosensitive plate, no satisfactory results can be obtained. In contrast, when the developer of the present invention is used, excellent results can be obtained in development and transfer of positively charged latent images.

The composite developer of the present invention also is advantageous in that at the development step both the developer components are consumed at the same speed and the composition is not changed while the development is repeated.

The present invention will now be described in detail with reference to the following Examples that by no means limit the scope of the invention. All of "parts" and "%" are by weight unless otherwise indicated.

#### EXAMPLE 1

A composition comprising 55 parts of agglomerated magnetite (Fe<sub>3</sub>O<sub>4</sub>) shown in Table 1, 37 parts of a styrene/butyl methacrylate copolymer (weight average molecular weight=27,000), 8 parts of low-molecular-weight polypropylene (average molecular weight=4,000) and 0.5 part of zinc stearate was kneaded and molten at 140° C. for 35 minutes by a two-roll kneading device. The kneaded composition was naturally cooled and roughly pulverized to a size of 0.5 to 2 mm by a cutting mill. Then, the roughly pulverized composition was finely pulverized by a jet mill and classified by a zigzag classifying machine to obtain a magnetic toner having a particle size within the range of from 5 to 35 microns. The classification was carried out

so that the lower limit of the particle size range was at least 2 times the particle size of magnetite.

TABLE 1

| Agglomerated Magnetite | Apparent Density (g/ml) | Number Average Particle Size ( $\mu$ ) | Coercive Force (Oe) | Saturation Magnetization (emu/g) | Residual Magnetization (emu/g) |
|------------------------|-------------------------|----------------------------------------|---------------------|----------------------------------|--------------------------------|
| A                      | 0.635                   | 1                                      | 148                 | 84.2                             | 10.6                           |
| B                      | 0.972                   | 3                                      | 54                  | 87.2                             | 5.1                            |
| C                      | 1.204                   | 5                                      | 100                 | 77.4                             | 8.6                            |
| D                      | 0.880                   | 7                                      | 90                  | 78.1                             | 8.0                            |

The values of the magnetic properties shown in Table 1 and subsequent Tables are those measured by using a magnetic property-measuring device supplied by Toei Kogyo (Model VSMP-1, magnetic field=5 K-Oe).

Separately, 55 parts of magnetite having a coercive force of 72 Oe, an apparent density of 0.40 g/ml and a particle size of 0.2  $\mu$ m, 41.5 parts of a thermoplastic resin (vinyl toluene/butadiene copolymer having a weight average molecular weight of 78,000), 0.675 part by weight of a negative charge controlling agent (Spirlon Black BHH supplied by Hodogaya Kagaku) and 3.5 parts of low-molecular-weight polypropylene were kneaded and molten in the same manner as described above. Classification was performed to collect particles having a particle size of from 5 to 25  $\mu$ m, and the particles were mixed with hydrophobic silica (R-972 supplied by Nippon Aerosil) in an amount of 0.2% based on the total amount to form a magnetic toner E. Each of the above-mentioned four magnetic toners (designated as magnetic toners A', B', C' and D') was dry-blended with the so-prepared magnetic toner E at a weight ratio of 70/30 to form composite toners A'', B'', C'' and D''.

The following copying test was carried out by using the so-prepared magnetic toners.

In a copying machine comprising a selenium drum (outer diameter=150 mm) as a photosensitive material, the intensity of a magnetic field on a developing sleeve (outer diameter=33 mm) having a magnet disposed therein through a non-magnetic member was adjusted to about 900 gauss, and the magnetic toner was applied to a developing roller of the so-called two-rotation system capable of rotating the magnet and the sleeve independently, while adjusting the distance between a spike-cutting plate and the sleeve to 0.3 mm. An arrangement was made so that the magnetic toner was supplied to the developing roller zone from a hopper. The distance between the surface of the photosensitive material and the developing roller was adjusted to 0.5 mm. The developing sleeve and photosensitive material were rotated in the same direction, and the magnet was rotated in the opposite direction. Under the foregoing conditions, charging (+6.7 KV), exposure, development, transfer (+6.3 KV), heater roller fixation and fur brush cleaning were performed. Slick paper having a thickness of 80  $\mu$ m was used as a transfer sheet, and the transfer speed was adjusted to 10 A4-1 size sheets per minute. The results of the copying test are shown in Table 2. The image density was measured on a solid black portion by using a commercially available reflective densitometer (supplied by Konishiroku Shashin Kogyo). A Copia test pattern supplied by Data Quest Co. was used as a copying test chart, and the gradient characteristic and resolving power were determined from a copy thereof. The sharpness was evaluated based on the line-image portion of the obtained copy and

when lines could be distinguished from one another definitely, the sharpness was judged as being excellent.

These magnetic toners A', B', C' and D' were characterized by a volume resistivity of  $1.2 \times 10^{14} \Omega\text{-cm}$  to  $4.6 \times 10^{14} \Omega\text{-cm}$  and a dielectric constant of 3.59 to 3.79 as measured under conditions of an electrode spacing of 0.65 mm, an electrode sectional area of  $1.43 \text{ cm}^2$  and an interelectrode load of  $105 \text{ g/cm}^2$ .

The magnetic toner E was characterized by a volume resistivity of  $1.5 \times 10^{14} \Omega\text{-cm}$  and a dielectric constant of 4.05 as measured under the above-mentioned conditions.

TABLE 2

|    | Magnetic Toner | Image Density | Background Density | Color Hue of Image | Sharpness         | Resolving Power (lines/mm) | Gradient Characteristic (steps) |
|----|----------------|---------------|--------------------|--------------------|-------------------|----------------------------|---------------------------------|
| 20 | A'             | 1.53          | 0.09               | bluish black       | good              | 8.0                        | 11                              |
|    | B'             | 1.54          | 0.10               | bluish black       | good to excellent | 8.0                        | 12                              |
| 25 | C'             | 1.50          | 0.09               | bluish black       | good to excellent | 8.0                        | 11                              |
|    | D'             | 1.30          | 0.10               | reddish black      | good to excellent | 7.1                        | 11                              |
| 30 | E              | 0.85          | 0.09               | black              | fair              | 6.3                        | 10                              |
|    | A''            | 1.63          | 0.09               | black              | good              | 8.0                        | 11                              |
|    | B''            | 1.65          | 0.09               | black              | excellent         | 8.0                        | 12                              |
|    | C''            | 1.65          | 0.09               | black              | excellent         | 8.0                        | 11                              |
|    | D''            | 1.50          | 0.09               | black              | excellent         | 7.1                        | 11                              |

## EXAMPLE 2

A composition comprising agglomerated magnetite (apparent density=0.785 g/ml, number average particle size=2.8  $\mu$ m, coercive force=58 Oe, saturation magnetization=87.2 emu/g, residual magnetization=5.1 emu/g), a thermoplastic resin (styrene/butyl methacrylate copolymer, weight average molecular weight=27,000) and high density polyethylene (average molecular weight=4,000) at a mixing ratio shown in Table 3 was treated in the same manner as described in Example 1 to form a magnetic toner having a particle size within a range of from 6 to 20  $\mu$ m.

TABLE 3

| Magnetic Toner | Mixing Ratio (parts)   |                     |                           |
|----------------|------------------------|---------------------|---------------------------|
|                | Agglomerated Magnetite | Thermoplastic Resin | High Density Polyethylene |
| F              | 75                     | 20                  | 5                         |
| G              | 65                     | 28                  | 7                         |
| H              | 55                     | 36                  | 9                         |
| I              | 45                     | 44                  | 11                        |
| J              | 35                     | 52                  | 13                        |

A composition comprising 55 parts of magnetite ( $\text{Fe}_3\text{O}_4$ ) shown in Table 4, 42 parts of a vinyl toluene/2-ethylhexyl acrylate copolymer (weight average molecular weight=139,000), 3.5 parts of a high density polyethylene wax (average molecular weight=4,000) and 0.5 part of calcium stearate was kneaded and molten. Classification was performed to collect particles having a particle size of from 5 to 20  $\mu$ m, and the particles were mixed with hydrophobic silica (R-972 supplied by Nippon Aerosil) in an amount of 0.2% based on the total amount.

TABLE 4

| Magnetite | Coercive Force (Oe) | Apparent Density (g/ml) | Particle Size ( $\mu$ )                    | Remarks             |
|-----------|---------------------|-------------------------|--------------------------------------------|---------------------|
| K         | 64                  | 0.40                    | 0.3-0.6                                    | cubic crystal       |
| L         | 350                 | 0.40                    | 0.5-0.6<br>(length)<br>0.06-0.1<br>(width) | needle crystal      |
| M         | 85                  | 0.37                    | 0.3-0.4                                    | cubic crystal       |
| N         | 134                 | 0.27                    | 0.27                                       | indeterminate-shape |

The so-prepared magnetic toners K', L', M' and N' were dry-blended with the above-mentioned magnetic toners F, G, H, I and J to obtain composite toners F', G', H', I' and J' shown in Table 5.

The following copying test was carried out by using the so-obtained magnetic toners.

In a copying machine comprising a selenium drum as a photosensitive material, the magnetic toner was applied to a developing roller having a magnetic disposed therein through a non-magnetic member while adjusting the distance between a spike-cutting plate and the developing roller to 0.3 mm. The distance between the surface of the photosensitive material and the developing roller was adjusted to 0.5 mm. The developing roller and photosensitive material were rotated in the same direction, but the moving speed of the developing roller was 2 times as high as the moving speed of the photosensitive material. Under the foregoing conditions, charging, exposure, development and heat fixation were performed. Slick paper having a thickness of 80  $\mu$ m was used as a transfer sheet. The transfer speed was adjusted to 10 A4-size sheets per minutes. The results of the copying test and the combinations of the magnetic toners are shown in Table 5. The image density was measured on a solid black portion.

TABLE 5

| Magnetic Toner         | Combination and Mixing Ratio of Magnetic Toners | Image Density | Background Density | Color Hue of Image | Sharpness (image quality) |
|------------------------|-------------------------------------------------|---------------|--------------------|--------------------|---------------------------|
| F' (present invention) | F/M', 30/70                                     | 1.41          | 0.09               | black              | good                      |
| G' (present invention) | G/N', 40/60                                     | 1.45          | 0.09               | black              | excellent                 |
| H' (present invention) | H/N', 90/10                                     | 1.57          | 0.10               | black              | excellent                 |
| I' (present invention) | I/K', 60/40                                     | 1.55          | 0.10               | black              | excellent                 |
| J' (present invention) | J/L', 40/60                                     | 1.52          | 0.12               | black              | good                      |
| F (comparison)         | —                                               | 0.50          | 0.09               | grayish black      | fair                      |
| G (comparison)         | —                                               | 1.28          | 0.09               | bluish black       | good                      |
| H (comparison)         | —                                               | 1.44          | 0.10               | bluish black       | good to excellent         |
| I (comparison)         | —                                               | 1.48          | 0.11               | bluish black       | good                      |
| J (comparison)         | —                                               | 1.45          | 0.20               | bluish black       | fair to good              |
| K' (comparison)        | —                                               | 1.40          | 0.10               | black              | good                      |
| L' (comparison)        | —                                               | 1.20          | 0.10               | black              | fair                      |
| M' (comparison)        | —                                               | 1.32          | 0.10               | black              | fair to good              |

TABLE 5-continued

| Magnetic Toner  | Combination and Mixing Ratio of Magnetic Toners | Image Density | Background Density | Color Hue of Image | Sharpness (image quality) |
|-----------------|-------------------------------------------------|---------------|--------------------|--------------------|---------------------------|
| N' (comparison) | —                                               | 1.21          | 0.10               | black              | fair                      |

## EXAMPLE 3

The magnetic toners A', B', C' and D' shown in Table 2 were used as the first developer component (A).

Separately, 55 parts of magnetic having a coercive force of 213 Oe, an apparent density of 0.55 g/ml and a particle size of 0.4 to 0.5  $\mu$ m, 41.5 parts of a thermoplastic resin (vinyl toluene/butadiene copolymer having a weight average molecular weight of 78,000), 0.675 part by weight of a negative charge controlling agent (Spiron Black BHH supplied by Hodogaya Kagaku), 0.45 part of zinc stearate and 3.5 parts of low-molecular-weight polypropylene were kneaded and molten in the same manner as described in Example 1. Classification was performed to collect particles having a particle size of from 5 to 25  $\mu$ m, and the particles were mixed with hydrophobic silica (R-972 supplied by Nippon Aerosil) in an amount of 0.2% based on the total amount to form a magnetic toner P. Each of the above-mentioned four magnetic toners (magnetic toners A', B', C' and D') was dry-blended with the so-prepared magnetic toner P at a weight ratio of 70/30 to form composite toners A'', B'', C'' and D''.

The following copying test was carried out by using the so-prepared magnetic toners.

In a copying machine comprising a selenium drum (outer diameter = 150 mm) as a photosensitive material, the intensity of a magnetic field on a developing sleeve (outer diameter = 33 mm) having a magnet disposed therein through a non-magnetic member was adjusted to about 900 gauss, and the magnetic toner was applied to a developing roller of the so-called two-rotation system capable of rotating the magnet and the sleeve independently, while adjusting the distance between a spike-cutting plate and the sleeve to 0.3 mm. An arrangement was made so that the magnetic toner was supplied to the developing roller zone from a hopper. The distance between the surface of the photosensitive material and the developing roller was adjusted to 0.5 mm. The developing sleeve and photosensitive material were rotated in the same direction, and the magnet was rotated in the opposite direction. Under the foregoing conditions, charging (+6.7 KV), exposure, development, transfer (+6.3 KV), heater roller fixation and fur brush cleaning were performed. Slick paper having a thickness of 80  $\mu$ m was used as a transfer sheet, and the transfer speed was adjusted to 30 A4-size sheets per minute. The results of the copying test are shown in Table 6. The image density was measured on a solid black portion by using a commercially available reflective densitometer (supplied by Kronishiroku Shashin Kogyo). A Copia test pattern supplied by Data Quest Co. was used as a copying test chart, and the gradient characteristic and resolving power were determined from a copy thereof. The sharpness was evaluated based on the line-image portion of the obtained copy and when lines could be distinguished from one another definitely, the sharpness was judged as being excellent.

When the composite magnetic toners according to the present invention were used, copies having a high image density and a clear and sharp image of a pure-black color were obtained at a copying speed of 30 sheets (A4-size sheets) without impairing the half tone-reproducing property or the resolving power.

TABLE 6

| Magnetic Toner  | Image Density | Back-ground Density | Color Hue of Image | Sharpness         | Re-solving Power (lines/mm) | Gradient Characteristic (stages) |
|-----------------|---------------|---------------------|--------------------|-------------------|-----------------------------|----------------------------------|
| A' (comparison) | 1.42          | 0.09                | bluish black       | good              | 8.0                         | 11                               |
| B' (comparison) | 1.43          | 0.10                | bluish black       | good to excellent | 8.0                         | 12                               |
| C' (comparison) | 1.40          | 0.09                | bluish black       | good to excellent | 8.0                         | 11                               |
| D' (comparison) | 1.39          | 0.10                | reddish black      | good to excellent | 7.1                         | 11                               |
| P (comparison)  | 0.72          | 0.09                | black              | fair              | 6.3                         | 10                               |
| A'''            | 1.58          | 0.09                | black              | excellent         | 8.0                         | 11                               |
| B'''            | 1.60          | 0.09                | black              | excellent         | 8.0                         | 12                               |
| C'''            | 1.61          | 0.09                | black              | excellent         | 8.0                         | 12                               |
| D'''            | 1.54          | 0.09                | black              | excellent         | 7.1                         | 12                               |

Note  
The toners A''', B''', C''' and D''' are included within the scope of the composite magnetic developer of the present invention.

## EXAMPLE 4

A composition comprising agglomerated magnetite (apparent density=0.785 g/ml, number average particle size=2.8 microns, coercive force=58 Oe, saturation magnetization=87.2 emu/g, residual magnetization=5.1 emu/g), a thermoplastic resin (styrene/acrylic copolymer, weight average molecular weight=71,000), zinc stearate and high density polyethylene (average molecular weight=4,000) at a mixing ratio shown in Table 7 was treated in the same manner as described in Example 1 to form a magnetic toner having a particle size within a range of from 6 to 20 microns.

TABLE 7

| Magnetic Toner | Mixing Ratio (parts)   |                      |                           |               |
|----------------|------------------------|----------------------|---------------------------|---------------|
|                | Agglomerated Magnetite | Thermo-plastic Resin | High Density Polyethylene | Zinc Stearate |
| Q              | 75                     | 20                   | 5                         | 0.5           |
| R              | 65                     | 28                   | 7                         | 0.5           |
| S              | 55                     | 36                   | 9                         | 0.5           |
| T              | 45                     | 44                   | 11                        | 0.5           |
| U              | 35                     | 52                   | 13                        | 0.5           |

A composition comprising 55 parts of magnetite ( $Fe_3O_4$ ) shown in Table 8, 42 parts of a vinyl toluene/2-ethylhexyl acrylate copolymer (weight average molecular weight=139,000), 3.5 parts of a high-density polyethylene wax, 0.6 parts of a negative charge controlling agent and 0.5 part of calcium stearate was kneaded and molten. Classification was performed to collect particles having a particle size of from 5 to 20 $\mu$ , and the particles were mixed with hydrophobic silica in an amount of 0.2% based on the total amount.

TABLE 8

| Magnetite | Coercive Force (Oe) | Apparent Density (g/ml) | Particle Size ( $\mu$ ) | Remarks                           |
|-----------|---------------------|-------------------------|-------------------------|-----------------------------------|
| V         | 135                 | 0.71                    | 0.1-0.2                 | indeterminate-shape cubic crystal |
| W         | 49                  | 0.47                    | 0.4                     | cubic crystal                     |

TABLE 8-continued

| Magnetite | Coercive Force (Oe) | Apparent Density (g/ml) | Particle Size ( $\mu$ ) | Remarks       |
|-----------|---------------------|-------------------------|-------------------------|---------------|
| X         | 56                  | 0.71                    | 0.5                     | cubic crystal |
| Y         | 90                  | 0.95                    | 0.47                    | cubic crystal |
| Z         | 200                 | 0.75                    | 0.5                     | cubic crystal |

10 The so-prepared magnetic toners V', W', X', Y' and Z' were dry-blended with the above-mentioned magnetic toners Q, R, S, T and U to obtain composite toners Q', R', S', T' and U' shown in Table 9.

15 The following copying test was carried out by using the so-obtained magnetic toners in the same manner as described in Example 3.

16 The obtained results are shown in Table 9. Incidentally, the image density was measured on a solid black portion.

20 By using the composite magnetic toner T', 10000 copies were formed by carrying out the copying operation continuously. In each of the obtained copies, the image density was higher than 1.52. In this case, the copying operation was conducted without fogging or reduction of the image density until the toner in the hopper was completely consumed. Thus, it was confirmed that the mixing toner of the magnetic toners T and W' was not changed during the copying operation because they were consumed at the same speed. From the results shown in Table 9, it is seen that when the composite toners of the present invention were used, the image density was improved over the image density attainable by single use of either of the two component even if the copying operation was carried out in a high-speed copying machine, and copied image generally excellent in the sharpness were obtained with reduction of fogging.

TABLE 9

| Magnetic Toner         | Combination and Mixing Ratio of Magnetic Toners | Image Density | Back-ground Density | Color Hue of Image | Sharpness (Image Quality) |
|------------------------|-------------------------------------------------|---------------|---------------------|--------------------|---------------------------|
| Q' (present invention) | Q/Y', 10/90                                     | 1.56          | 0.09                | black              | excellent                 |
| R' (present invention) | R/V', 40/60                                     | 1.53          | 0.09                | black              | excellent                 |
| S' (present invention) | S/X', 90/10                                     | 1.59          | 0.10                | black              | excellent                 |
| T' (present invention) | T/W', 60/40                                     | 1.52          | 0.10                | black              | excellent                 |
| U' (present invention) | V/Z', 30/70                                     | 1.58          | 0.12                | black              | excellent                 |
| Q (comparison)         | —                                               | 0.41          | 0.09                | grayish black      | fair                      |
| R (comparison)         | —                                               | 0.10          | 0.09                | bluish black       | good                      |
| S (comparison)         | —                                               | 1.36          | 0.10                | bluish black       | good to excellent         |
| T (comparison)         | —                                               | 1.37          | 0.11                | bluish black       | good                      |
| U (comparison)         | —                                               | 1.32          | 0.18                | bluish black       | fair to good              |
| V (comparison)         | —                                               | 1.23          | 0.10                | black              | good                      |
| W (comparison)         | —                                               | 1.27          | 0.10                | black              | good                      |
| X (comparison)         | —                                               | 1.26          | 0.10                | black              | good                      |
| Y (comparison)         | —                                               | 1.33          | 0.10                | black              | good                      |
| Z (comparison)         | —                                               | 1.28          | 0.10                | black              | good                      |

What is claimed is:

1. A dry composite magnetic developer for electro-photography which comprises a mixture of (A) a first particulate shaped article of a composition comprising a binder resin medium and a non-pulverizing agglomerate of cubic particles of magnetite wherein numerous fine particles of magnetite are so densely aggregated with one another that the particle size distribution is not substantially changed even after ball-milling for five hours' treatment, said agglomerate having a number average particle size of 2 to 10 microns as measured by an electron microscope and an apparent density of 0.5 to 1.5 g/m as measured according to the method of JIS K-5101, and (B) a second particulate shaped article of a composition comprising a binder resin medium and fine magnetite particles having a particle size of 0.2 to 1 micron, each of the agglomerate in the component (A) and the fine magnetite in the component (B) being present in an amount of 35 to 75% by weight based on the sum of the amounts of the binder resin medium and the magnetite material, the component (A) and the component (B) being present at an (A)/(B) weight ratio of from 95/5 to 10/90, said component (A) having a number average particle size of 5 to 35 microns, said component (B) having a number average particle size of 5 to 30 microns.

2. A magnetic developer as set forth in claim 1 wherein the binder resin medium comprises a homopolymer or copolymer of at least one mono- or di-ethylenically unsaturated monomer selected from the group consisting of vinyl aromatic monomers and acrylic monomers.

3. A magnetic developer as set forth in claim 2 wherein said binder resin medium has a volume resistivity of at least  $1 \times 10^{15} \Omega\text{-cm}$ .

4. A dry composite magnetic developer as set forth in claim 3 wherein the non-pulverizing agglomerate has a number average particle size of 2 to 7 microns and an apparent density of 0.7 to 1.3 g/ml and is further characterized by a saturation magnetization of 75 to 88 emu/g, a residual magnetization of 3 to 12 emu/g and a coercive force of 40 to 150 Oe.

5. A dry composite magnetic developer according to claim 4 wherein the fine magnetite particles in the sec-

ond particulate shaped article (B) have a particle size of from 0.3 to 0.8 microns.

6. A dry composite magnetic developer according to claim 5 wherein the fine magnetite particles in the second particulate shaped article (B) have an apparent density larger than 0.45 g/ml and consists of cubic particles or rounded intermediate-shaped particles and have a shape anisotropy, defined as the ratio of the maximum size to the minimum size, of from 1.0 to 5.5.

7. A magnetic developer as set forth in claim 6 wherein the amount of the agglomerate in component (A) and the amount of the fine magnetite in the component (B) are each in the range of from about 40 to 70% by weight, based on the sum of the amounts of the binder resin medium and the magnetite material.

8. A magnetic developer as set forth in claim 7 wherein component (A) and component (B) are present at an (A)/(B) weight ratio of 95/5 to 30/70.

9. A magnetic developer as set forth in claim 1, wherein the agglomerate has a saturation magnetization of 75 to 88 emu/g, a residual magnetization of 3 to 12 emu/g and a coercive force of 40 to 150 Oe.

10. A magnetic developer as set forth in claim 1, wherein the agglomerate has the substantially same configuration as that shown in an electron microscope photograph of FIG. 1 of the accompanying drawings.

11. A magnetic developer as set forth in claim 1, wherein the first particulate shaped article (A) and the second particulate shaped article (B) are present at an (A)/(B) weight ratio of from 95/5 to 30/70.

12. A magnetic developer as set forth in claim 11, wherein the fine magnetite in the second particulate shaped article (B) has an apparent density larger than 0.45 g/ml.

13. A magnetic developer as set forth in claim 11, wherein the fine magnetite in the component (B) consists of cubic particles or rounded indeterminate-shape particles.

14. A magnetic developer as set forth in claim 11, wherein the fine magnetite in the component (B) has a shape anisotropy, defined as the ratio of the maximum size to the minimum size, of from 1.0 to 5.5.

\* \* \* \* \*